

## UNITED STATES PATENT OFFICE.

JOHN I. CRAETREE AND GLENN E. MATTHEWS, OF ROCHESTER, NEW YORK, ASSIGNEES TO EASTMAN KODAK COMPANY, OF ROCHESTER, NEW YORK, A CORPORATION OF NEW YORK.

## PHOTOGRAPHIC BATH.

No Drawing.

Application filed May 6, 1925. Serial No. 23,499.

Our invention relates to photographic processes and more particularly to a method of indicating, under the light conditions necessary in a photographic dark room, 5 when the acidity of baths whose usefulness is at least partly dependent upon their acidity approaches a limiting value.

We have found that the change, which is not ordinarily easily detectable, can be noted 10 promptly if there is added to the bath an indicator which is selected, not only by the degree of acidity at which it changes color, but also by the differentiation between its colors under the light of definitely limited 15 wave length by which it must be inspected.

It is not sufficient that the apparent colors are different when viewed by daylight since the same apparent color sensation may be obtained by different combinations of light 20 of different wave lengths; and it can easily happen that two colors appearing quite different by daylight may look the same under the light of selected wave lengths which happen to be common to both. It is therefore 25 necessary to choose an indicator which has markedly different transmissive properties for light waves in the orange and red portions of the spectrum. Certain indicators having the property of indicating 30 a change at approximately the point useful in rinse and fixing baths are di-bromo-thymol-sulfon-phthalein, known as brom thymol blue, which by daylight changes from yellow to blue and has a range between pH 35 values of 6.0 and 7.6; archil or orchil which changes from pink to lilac between 5.6 and 7.6; phenol-nitro-sulfon-phthalein which changes from yellow to purple between 6.6 and 8.4 and di-bromo-ortho-cresol-sulfon-phthalein, known as brom cresol purple, 40 which changes from yellow to purple between 5.2 and 6.8.

Other indicators for other ranges of acidity which are useful in other baths and 45 which also have two markedly different sets of transmissive properties to light in the orange and red portions of the spectrum are: tetra-bromo-phenol-sulphon-phthalein, known as bromo phenol blue, and tetra-chloro-phenol sulfon phthalein, both changing from yellow to blue in the range between 5.0 and 4.6; tetra-bromo-m-cresol-sulfon phthalein, known as brom cresol green, whose range is between pH values of 4.0

and 5.5, and which in daylight changes from 55 yellow to blue; and cochineal, whose range is between pH values of 4.8 and 6.2 and which changes from yellow to lilac by daylight, and lacmosol or resorcin blue, changing from red to blue between 4.4 and 5.5. 60

In processing photographic papers, an acid rinse bath or "stop bath" is frequently used between development and fixation. An acid rinse bath is used to neutralize the alkaline developer carried over on the surface 65 of the photographic print and thus prevent further progress of development, and to avoid carrying alkaline developer into the fixing bath. This is particularly undesirable when the latter contains alum as it then 70 precipitates a sludge when in an alkaline condition and stains the photographic paper.

A typical formula which complies with the requirements outlined above with reference to a stop bath is the following:

|                         | Parts. |
|-------------------------|--------|
| Water                   | 1000   |
| Acetic acid (28% pure)  | 45     |
| Brom thymol blue (0.04) | 25 80  |

The brom thymol blue solution should have 3.2 cc. of N/20 sodium hydroxide solution added per 0.1 gram of indicator.

An indicator for use with an alum fixing 85 bath must be selected so as to change color just previous to the point where the fixing bath would either tend to stain the emulsion or precipitate a sludge. A typical formula which complies with these requirements is 90 the following: Sodium sulphite (desiccated), 12 grams; potassium alum (aluminium and potassium sulphate), 13 grams; citric acid, 6 grams; hypo (sodium thiosulphate), 240 grams; brom thymol blue (0.04%), 25 c.c.; 95 water to make 1 liter. The brom thymol blue solution should have 3.2 cc. of N/20 sodium hydroxide solution added per 0.1 grams of indicator. The above amounts would make only a small quantity but it is 100 to be understood that they represent merely the proportions of the ingredients.

Having thus described our invention, what we claim as new and desire to secure by Letters Patent is:

1. The method of indicating when a bath, useful in photographic processes carried out in light of certain definite limited wave

lengths, approaches a predetermined acidity affecting its usefulness that comprises incorporating therein an indicator that causes the color of the bath to change as it ap-

5 proaches such acidity, the original and final colors of the bath being ones that are sharply differentiated when viewed by light of said wave lengths.

2. The method of indicating when a bath, 10 useful in photographic processes carried out in light of wave lengths in the orange and red portions of the spectrum, approaches a predetermined acidity affecting its usefulness that comprises incorporating therein 15 an indicator that causes the color of the bath to change as it approaches such degree of acidity, the light transmission character-

istics of the bath before and after the color change being markedly different to light waves in the orange and red portions of the 20 spectrum.

3. A bath intended for use after development in a photographic process and containing an indicator whereby the color of the bath will change in the vicinity of  $pH=6.5$ , 25 the light transmission characteristics of the bath before and after the color change being markedly different to light waves in the orange and red portions of the spectrum.

Signed at Rochester, New York this 2nd 30 day of May, 1925.

JOHN I. CRABTREE.  
GLENN E. MATTHEWS.